

May 9, 1944.

H. R. HOUCHINS

2,348,474

POROUS ABRASIVE ARTICLE

Filed Feb. 2, 1942

2 Sheets-Sheet 1

*Fig. 1.*



*Inventor*  
Henry R. Houchins

*by* *W.C. Polley*  
Attorney

May 9, 1944.

H. R. HOUGHINS

2,348,474

POROUS ABRASIVE ARTICLE

Filed Feb. 2, 1942

2 Sheets-Sheet 2



Fig. 2.



Fig. 3.



Fig. 4.

Inventor  
Henry R. Houchins

by *W. Dole*  
Attorney

Patented May 9, 1944

2,348,474

# UNITED STATES PATENT OFFICE

2,348,474

## POROUS ABRASIVE ARTICLE

Henry R. Houchins, Niagara Falls, N. Y., assignor  
to The Carborundum Company, Niagara Falls,  
N. Y., a corporation of Delaware

Application February 2, 1942, Serial No. 429,288

14 Claims. (Cl. 51—308)

The invention of this application relates to the formation of abrasive wheels and particularly to abrasive wheels of the type known as "snagging" wheels, which are used for rough grinding in the removal of irregularities from the surfaces of castings.

It is one of the objects of the present invention to produce a wheel with the maximum density compatible with fast grinding action, but without the use of fine abrasive particles to fill the spaces between the larger abrasive grains. Other objects of the invention are to obtain comparatively high porosity in an abrasive wheel while maintaining high density and high strength, to produce an abrasive wheel containing the maximum possible number of active abrasive grains per unit of grinding area, and to avoid breaking the large grains of abrasive.

It is at present customary to manufacture snagging wheels by pressing a damp mixture of abrasive and bond. The mixture contains a rather high proportion of bond and a long range of sizes of abrasive particles in order to obtain sufficient density to cause resistance to wear in the hard service to which such wheels are subjected. The cutting rate of snagging wheels made according to this procedure is adversely affected, however, since the long range of grit sizes and the comparatively large quantity of finer grains reduces the number of active abrasive grains available in the surface of the abrasive wheel. In addition, the high percentage of bond necessarily produces a separation of the abrasive grains and fills up a considerable part of the space between the grains. Snagging wheels made by the method described above thus have a tendency to fill rapidly and become glazed when in use.

By the method of the present invention the defects of snagging wheels produced by the practice described above are corrected and wheels having higher cutting rates and little tendency to fill or become glazed may be easily produced.

In the accompanying drawings, Figure 1 is a somewhat diagrammatic view of one form of apparatus which may be used in carrying out the process of the present invention. Figure 2 is a photomicrograph of the structure of an abrasive wheel made according to the method of the present invention. Figures 3 and 4 are photomicrographs of the structure of abrasive wheels produced by the pressing method previously in use.

A description of the method of this invention will be made with reference to Figure 1 of the drawings. In Figure 1, 10 represents a tank

5 or vat in which is contained a slip or slurry 11 of a ceramic bonding material. A ring or tube 12, of metal or other suitable material, is provided with lugs 13 near the bottom thereof and extending inwardly. Resting upon lugs 13 is a perforated plate or disc 14 on which rests a fine screen 15, adapted to support a body or mass of abrasive 16. Resting upon abrasive grain 16 is another screen 17 and a perforated plate or disc 18. Tube or ring 12 may conveniently be and is preferably split, as at 19, to facilitate the removal of the abrasive wheel after it is formed.

In carrying out the present invention with the apparatus shown in Figure 1, a suitable ceramic bond is chosen and the ingredients thereof are formed into a slip or slurry with water. This slip is placed in vat 10. Abrasive grain of the desired character and size is placed in tube 12 between plates 14 and 18 and screens 15 and 17. The grain after being put in tube 12 is in what may be called a vertically self-supporting condition. Each grain must necessarily contact at least one other grain thus to be held in position. After the top screen 17 and top plate 18 are placed on top of the abrasive grain, the abrasive grain is compacted by any suitable means. A convenient and satisfactory method of compacting the abrasive grain is by subjecting the tube 12 containing the abrasive grain to vibration.

20 30 When a mix of abrasive grain and bond is pressed in the normal manner of the prior art many of the larger grains are crushed and thus rendered less effective. By the present method of initially compacting the grain to maximum density all danger of crushing or breaking the grain is avoided and the grain is, to a considerable extent, formed into an inter-locking structure. Greater abrasive density can thus be obtained than by the old methods of pressing or 35 puddling where bond keeps the abrasive grains apart. Vibration may also have some tendency to orient the grain toward the periphery of tube 12.

40 Ring or tube 12 containing the compacted grain is then slowly lowered into tank or vat 10 containing the slip 11 of ceramic bond and the slip is allowed to penetrate upwardly through the compacted mass of grain, the tube being prevented from resting directly on the bottom of vat 10 by feet 20, conveniently formed integrally with the sides thereof. The hydrostatic pressure of the slip which surrounds tube 12 is usually sufficient to cause the slip or slurry to rise in tube 12 and displace the air from the compacted grain. If necessary to prevent displace-

ment thereof the covering screen 17 and plate 18 may be clamped in place or held down by a weight (not shown).

After the abrasive grain has been saturated with the slurry of bonding material it is withdrawn from vat 10, suitable precautions being taken to prevent drainage of the slurry from the grain, and dried. It is thereafter burned or fired in the usual manner, depending upon the type of abrasive grain and bond.

As previously mentioned, the hydrostatic pressure of the slurry in vat 10 surrounding tube 12 is usually sufficient to cause the slurry to permeate the compacted mass of grain. In cases where, because of the use of finer abrasive particles, a slip of high viscosity, or for other reasons, penetration of the grain by the slurry is difficult or imperfect it has been found possible to increase the speed and completeness of penetration in several ways. A preliminary treatment of the abrasive grain with a wetting agent has been found very advantageous. Subjecting tube 12 to vibration while it is immersed in vat 10 also hastens saturation of the granular mass with the slurry. If necessary, a bonnet or hood (not shown) can be attached to the top of tube 12 and a slight reduction of pressure therein be employed to aid in penetration of the granular mass by the slurry.

The amount of bond in a wheel made by the method of the present invention, other variable factors being constant, is a function of the specific gravity of the bonding slip or slurry. Since this specific gravity may be easily adjusted by varying the proportions of bond and water, the amount of bond in the wheel, and hence the hardness of the wheel, may be readily varied.

The following are typical examples of abrasive wheels made by this process.

#### Example I

Grain size distribution: Parts by weight  
 16 grit silicon carbide..... 15  
 20 grit silicon carbide..... 55  
 24 grit silicon carbide..... 20  
 36 grit silicon carbide..... 10

Bond composition: Parts by weight  
 Feldspar ..... 60  
 Kaoline ..... 15  
 Ball clay ..... 15  
 Flint ..... 9  
 Talc ..... 1

The abrasive grain is mixed thoroughly and placed in a tube or ring, such as that shown at 12 in Figure 1, of the proper diameter and is vibrated until it reaches its highest density, which is usually obtained after  $\frac{1}{2}$  to 1 minute of vibration.

The bond ingredients are mixed and formed into a slip by mixing 100 parts by weight of bond with 66.5 parts by weight of water. The slip is then deflocculated to the greatest possible degree with the necessary amount of a 50% sodium silicate solution. The amount of silicate necessary is, in general, of the order of .25 percent of the amount of dry bond. The resulting slip should have a specific gravity of 1.56.

The tube or ring containing the compacted grain is then lowered into the slip and allowed to sit therein until the slip covers the surface of upper plate 18. Obviously, the level of the slip 11 in vat 10 must be higher than plate 18

with tube 12 in position in vat 10. The tube or ring containing the abrasive grain saturated with slip is then withdrawn from the vat containing the slip or slurry of bond, dried at 325° F., shaved to size and shape, and burned or fired in a kiln at cone 12. Following the burning, the wheel is finished in the usual way. A wheel made in accordance with this example contains about 17% bond by weight. By increasing the specific gravity of the slip, wheels having as much as 22% bond have been produced.

The following example exemplifies the formation of a snagging wheel using fused alumina abrasive.

#### Example II

Grain size distribution: Parts by weight  
 14 grit fused alumina..... 50  
 16 grit fused alumina..... 25  
 20 grit fused alumina..... 25

Bond composition:  
 Albany slip clay.

The granular abrasive after being thoroughly mixed together is placed in a ring or tube of the proper diameter and, if desired, is compacted as above described in Example I by the use of vibration. The tube containing the mass of grain is then lowered into a vat in which there is a slurry or suspension of the Albany slip clay which has been made up with water to a specific gravity of 1.42. Suspension of the clay is maintained by the use of a small amount of suitable deflocculating agent such as, for example, a solution of sodium silicate. After the clay slurry has saturated the mass of grain, the tube containing the grain is withdrawn from the vat, dried at a moderate temperature, for example 300° F., and then, after being shaved to size and shape, burned or fired at approximately 1200° C.

The wheel produced by Example II is, as is customary with alumina snagging wheels, somewhat less hard and dense than the silicon carbide wheel produced by Example I. Of course the density and hardness of the wheel could be increased by suitably varying the grit size of the abrasive, its degree of compactness or the specific gravity of the clay slurry and hence the amount of bond in the wheel.

As will be evident, the invention of the present application is applicable to abrasive materials of various kinds and may be employed with ceramic bonds of varying composition as well as other types of bonds so long as the bonding ingredients are adapted for use as a slurry or dispersion.

It has been found through tests that abrasive articles made by the method of the present invention have very much greater transverse strength and resistance to impact than abrasive articles of the same composition, pressed in the manner of the prior art. At the same time, the abrasive articles made by the present method have greater density, reflected in lower porosity and absorption, than pressed abrasive articles of the same composition.

The improved strength of abrasive articles made by the method of this invention is indicative of a better distribution of the bond in the abrasive article, and this indication is supported by photomicrographs made of sections of such articles.

In Figure 2 is shown such a photomicrograph, and it may be seen from this figure that the bond is distributed as more or less continuous

films between adjacent grains of abrasive, leaving the open spaces between the grains relatively free of bond. It is believed that this distribution of the bond is obtained by reason of the fact that the bond slurry with which the grain is saturated, upon drying, shrinks away from the center of the intergranular spaces into the finer channels between the grains, thus bonding the grains more firmly while leaving the intergranular spaces open, and giving an article with sufficient evenly distributed pores as to minimize loading and glazing when in use. Because the mass of grain is in a vertically self-supporting condition, as has been explained above, before being penetrated or permeated by the slip of ceramic bond and because the abrasive grains in the mass are not substantially displaced by the penetration of the bond slip, the grains in the finished bonded abrasive article are supported by each other in a state of substantial equilibrium in a vertical direction. That is, with suitable side support for the grains on the outer side surface of the article such as was initially furnished the grains in the mass by the sides of the porous container 12, and a suitable bottom support for the grains conforming to the bottom surface of the article, even if the bond of the finished article were removed the grains would remain in substantially the same position which they have in the finished article.

In Figure 3 is shown a photomicrograph of a section of an abrasive snagging wheel formed by the molding method commonly used and containing what is a common percentage of bond in commercial snagging wheels—25% by weight. It will be seen from this figure that the proportion of large, effective grains is much smaller than in Figure 2 and that the bond occupies a considerable number of the intergranular spaces, thus reducing the effectiveness of the wheel so far as porosity is concerned.

In Figure 4 is shown a photomicrograph of a section of an abrasive snagging wheel which has been molded in the common manner, but which contains only approximately 17% by weight of bond. It will be noted, in this figure, that the proportion of small, ineffective grains is large and that the bond is not as effectively located as in Figure 2. Apparently a considerable amount of the bond is clinging to surfaces of the abrasive grains which are not in contact, and is thus not effective in bonding.

In general, it may be said that the structures shown in Figures 3 and 4 are similar in that the effective grain area is smaller in both cases than in Figure 2. Moreover, the bond in Figure 2 is effectively distributed, while, in Figure 3, it occupies too much of the intergranular space, and in Figure 4, furnishes insufficient bonding effect. Comparison of these photomicrographs will make it clear that the structure produced by the present invention is markedly different from the structure of abrasive wheels produced by the older pressing method.

While there has been described a way of producing abrasive wheels by allowing the penetration upward through a mass of grain of a slurry of bond ingredients, it must not be assumed that this is the only method by which the improved articles of the present invention may be produced. While the upward penetration is convenient, since it makes it easier for air to escape from the mass of grain, satisfactory articles can be obtained by other means. Thus the bond slurry may be poured into a mold con-

taining abrasive grain suitably compacted, and a structure similar to that above described will be produced. Of course, precautions must be taken to prevent the entrapment of air in the mass of grain and slurry, and it may be desirable to vibrate the mold during pouring of the slurry, to assist the escape of air.

The superiority of snagging wheels made by the process of the present invention is shown by the fact that their cutting rates are, in general, about twice that of snagging wheels of commercial types made by prior art methods, when grinding the same material under the same conditions.

While the present invention has been described particularly with respect to the manufacture of snagging wheels, it will be recognized that other types of abrasive articles and wheels can be easily and conveniently made by this process, and it is not intended that the invention shall be limited to use in the making of snagging wheels.

Where "vibration" has been referred to in this specification and claims, it is meant to include not only high-frequency vibration such, for example, as that induced by electromagnetic vibrators and the like, but also to include hammering, jolting and other low-frequency vibrating methods.

The above-described invention is intended to be covered by this application as set forth in the appended claims, and it is not intended that the invention shall be limited except by those claims.

I claim:

1. The improved process of making abrasive snagging wheels which comprises: treating abrasive grain of relatively large grit size with a wetting agent; placing the treated abrasive grain in a porous container; compacting said abrasive grain by subjecting it to vibration; forming a ceramic bond raw mix into a slurry with water; deflocculating said slurry; immersing said abrasive grain in the deflocculated slurry so as to allow upward penetration and saturation of the compacted grain by said slurry; subjecting the container holding the grain to vibration while said abrasive grain is immersed in said slurry; drying the saturated mass of abrasive grain; and burning the dried product to at least partially vitrify the bond.
2. The improved process of making abrasive snagging wheels which comprises: treating abrasive grain of relatively large grit size with a wetting agent; placing the treated abrasive grain in a porous container; compacting said abrasive grain by subjecting it to vibration; forming a ceramic bond raw mix into a slurry with water; deflocculating said slurry; immersing said abrasive grain in the deflocculated slurry so as to allow upward penetration and saturation of the compacted grain by said slurry; drying the saturated mass of abrasive grain; and burning the dried product to at least partially vitrify the bond.
3. The improved process of making abrasive snagging wheels which comprises: placing abrasive grain of relatively large grit size in a porous container; compacting said abrasive grain by subjecting it to vibration; forming a ceramic bond raw mix into a slurry with water; deflocculating said slurry; immersing said abrasive grain in the deflocculated slurry so as to allow upward penetration and saturation of the compacted grain by said slurry; subjecting the container holding the grain to vibration while said abrasive grain is immersed in said slurry; drying the

saturated mass of abrasive grain; and burning the dried product to at least partially vitrify the bond.

4. The improved process of making abrasive snagging wheels which comprises: placing abrasive grain of relatively large grit size in a porous container; compacting said abrasive grain by subjecting it to vibration; forming a ceramic bond raw mix into a slurry with water; immersing said abrasive grain in the slurry so as to allow upward penetration and saturation of the compacted grain by said slurry; drying the saturated mass of abrasive grain; and burning the dried product to at least partially vitrify the bond.

5. The improved process of making abrasive articles which comprises: treating abrasive grain with a wetting agent; placing said treated abrasive grain in a porous container; compacting said abrasive grain by subjecting it to vibration; forming a ceramic bond raw mix into a slurry with water; deflocculating said slurry; immersing said abrasive grain in the deflocculated slurry so as to allow upward penetration and saturation of the compacted grain by said slurry; subjecting the container holding the grain to vibration while said abrasive grain is immersed in said slurry; drying the saturated mass of abrasive grain; and burning the dried product to at least partially vitrify the bond.

6. The improved process of making abrasive articles which comprises: treating abrasive grain with a wetting agent placing said treated abrasive grain in a porous container; compacting said abrasive grain forming a ceramic bond raw mix into a slurry with water; deflocculating said slurry; immersing said abrasive grain in the deflocculated slurry so as to allow upward penetration and saturation of the compacted grain by said slurry; drying the saturated mass of abrasive grain; and burning the dried product to at least partially vitrify the bond.

7. The improved process of making abrasive articles which comprises: placing abrasive grain in a porous container; compacting said abrasive grain; forming a slurry of bonding ingredients with water; deflocculating said slurry; immersing said abrasive grain in the deflocculated slurry so as to allow upward penetration and saturation of the compacted grain by said slurry; drying the saturated mass of abrasive grain; and maturing the dried product.

8. The improved process of making abrasive articles which comprises: placing abrasive grain in a porous container; compacting said abrasive grain; forming a slurry of bonding ingredients with water; introducing said slurry into said porous container so as to saturate the compacted grain therewith; drying the saturated mass of abrasive grain; and maturing the dried product.

9. The improved process of making abrasive articles which comprises: placing abrasive grain in a porous container; forming a fluid dispersion of bonding ingredients; introducing said dispersion into said porous container so as to saturate the abrasive grain therewith; drying the sat-

urated mass of abrasive grain; and maturing the dried product.

10. The improved process of making abrasive articles which comprises: compacting a mass of abrasive grain; forming a fluid dispersion of bonding ingredients; saturating the compacted grain with said dispersion; and drying and curing the saturated mass of abrasive grain.

11. The improved process of making abrasive articles which comprises placing a quantity of abrasive grains of relatively large grit size and lying within a short range of grit sizes in such a manner that they form a vertically self-supporting mass, said abrasive grains being in intimate contact with each other, thereafter saturating the mass of abrasive grain with a fluid dispersion of ceramic bond without substantially changing the disposition of the abrasive grains relative to each other, drying the saturated mass of abrasive grain, and burning the dried product to at least partially vitrify the ceramic bond, whereby the bonding material is distributed as more or less continuous films between adjacent grains of abrasive, there being open spaces between the grains, said open spaces being relatively free of bond.

12. A dense ceramic bonded snagging wheel comprising abrasive grains and matured ceramic bonding material, the abrasive grains in the article being of relatively coarse grain sizes and lying within a short range of grain sizes, each grain contacting a sufficient number of other grains in the wheel to be supported in substantial vertical equilibrium in the absence of bonding material, said matured bonding material being distributed substantially uniformly upon the abrasive grains as more or less continuous films within the pore spaces existing between the abrasive grains.

13. A dense ceramic bonded abrasive article comprising abrasive grains and matured ceramic bonding material, the abrasive grains in the article being of relatively coarse grain sizes and lying within a short range of grain sizes, each grain contacting a sufficient number of other grains in the article to be supported in substantial vertical equilibrium in the absence of bonding material, said matured bonding material being distributed substantially uniformly upon the abrasive grains as more or less continuous films within the pore spaces existing between the abrasive grains.

14. A dense ceramic bonded abrasive article comprising abrasive grains and matured ceramic bonding material, the abrasive grains in the article being of relatively coarse grain sizes, each grain contacting a sufficient number of other grains in the article to be supported in substantial vertical equilibrium in the absence of bonding material, said matured bonding material being distributed substantially uniformly upon the abrasive grains as more or less continuous films within the pore spaces existing between the abrasive grains.